

# United States Patent [19]

Immel

[11] 3,923,613

[45] Dec. 2, 1975

[54] ACIDIC GALVANIC COPPER BATH

[75] Inventor: **Waldemar Immel**, Solingen,  
Germany

[73] Assignee: **W. Kampschulte & Cie.**, Solingen,  
Germany

[22] Filed: Sept. 27, 1974

[21] Appl. No.: 510,025

**Related U.S. Application Data**

[63] Continuation of Ser. No. 334,296, Feb. 21, 1973,  
abandoned.

[30] **Foreign Application Priority Data**

Feb. 22, 1972 Germany..... 2208198

[52] U.S. Cl..... 204/52 R

[51] Int. Cl.<sup>2</sup>..... C25D 3/38

[58] **Field of Search**..... 204/52 R, 44, 106

[56] **References Cited**

UNITED STATES PATENTS

|           |         |                    |            |
|-----------|---------|--------------------|------------|
| 2,828,252 | 3/1958  | Fischer.....       | 204/52 R X |
| 2,910,413 | 10/1959 | Strauss et al..... | 204/44     |
| 3,414,493 | 12/1968 | Nobel et al.....   | 204/52 R   |
| 3,704,213 | 11/1972 | Fournier .....     | 204/52 R   |

*Primary Examiner*—G. L. Kaplan

*Attorney, Agent, or Firm*—Walter Becker

[57] **ABSTRACT**

An acidic galvanic copper bath of customary composition with organic sulfonic acids or the salts thereof as basic luster substances and/or with anion active and/or non-ionogenic wetting agents, in which the bath includes substituted urea derivatives.

**3 Claims, No Drawings**

## ACIDIC GALVANIC COPPER BATH

This application is a continuation of U.S. application Ser. No. 334,296 filed on Feb. 21, 1973, which is now abandoned.

The present invention relates to an acidic galvanic high luster copper bath of the customary composition with a content in organic sulfonic acids or the salts thereof as basic lustering agent and/or a content in anionactive and/or nonionogenic wetting agents.

Acidic high luster copper baths permit the separation



or precipitation of high luster copper deposits which with various types of baths are also well flattened. The acidic copper deposits are ductile, free from pores and yield a very good corrosion protection. A particular advantage of the acidic high luster copper baths is seen in their great economy, low working temperatures and the simple detoxication or decontamination with regard to the removal of cyanogen. The addition of the luster and flattening substances is generally effected in conformity with the measured or calculated Ampere hours.

It is known in acidic galvanic copper baths of customary composition with a content in organic sulfonic acids for purposes of obtaining a flattening effect to employ such derivatives of thiourea which in the molecular bond in addition to the thiourea component also comprise one or more groups in which the carbon atom is bonded exclusively to heteroatoms, such as sulfur and nitrogen. These organic sulfonic acids impart upon the baths intermixed therewith flattening properties, but as chemical compounds on the thiourea basis they have the drawback that, when the acidic copper electrolyte is left standing without current passing therethrough, the sulfonic acids will in view of their thiourea/Isothiourea tautomerism with regard to their reactive SH-grouping be strongly subjected to selfdisintegration. As a further drawback it has been found that such baths have only a low concentration-dependent tolerance as to action.

It is, therefore, an object of the present invention to overcome the above mentioned drawbacks of the heretofore known acidic galvanic copper baths without affecting the deposit of the high luster and well flattened copper precipitation.

This object has been realized according to the present invention by the fact that the bath instead of containing the thiourea component contains the urea component which tends considerably less to tautomerism

and which is built into the molecule of the sulfonic acids or the salts thereof. Preferably, the copper bath according to the present invention is characterized by an additional content in N-mono and/or di/urea substituted with alkylmercapto groups. Expediently, the copper bath contains the substances which are employed as flattening and lustering agents in conformity with the present invention in quantities of from  $5 \cdot 10^{-4}$  to  $2 \cdot 10^0$  g/l, preferably from  $3 \cdot 10^{-3}$  to  $7 \cdot 10^{-2}$  g/l. As examples for such compounds according to the invention there may be mentioned:

35 As an example for explaining an acidic galvanic high luster copper bath according to the invention, by means of which the drawbacks of the above described state of the art are eliminated and by means of which flattening grades in excess of 50% can be realized without the breakdown of the bath, the following is set forth. The bath is accordingly characterized by a high tolerance as to its effectiveness in conformity with great concentrations.

## EXAMPLE

45 200 g/l copper sulfate  
55 g/l sulfuric acid  
50 mg/l chlorine ions  
120 mg/l N,N-dipropylthiocarbamide acid propylester  
w-sodium combined with a sulfo acid  
6 mg/l (hexamethyledithiocarbamylmethylene)-urea  
1 g/l non-ionogenic wetting agent  
working temperature 20 - 30°C  
current density 0.75 - 5.5 Amp/dm<sup>2</sup>

55 When copper plating prenickel plated steel sheet metal with a starting rough depth of  $0.6 \mu$  m, with a current density of from 5 Amp/dm<sup>2</sup> there is obtained a lustrous copper layer or coating with a flattening of approximately 60%. The bath may be operated with and without air.

60 It is, of course, to be understood that the present invention is, by no means, limited to the specific example set forth above but also comprises any modifications within the scope of the appended claims.

What I claim is:

65 1. In an acidic galvanic copper bath the improvement comprising providing the bath with a substituted urea selected from the group consisting of



25

2. A copper bath of claim 1 wherein the substituted urea is present in an amount from  $5 \times 10^{-4}$  to 2 grams per liter.

3. A copper bath of claim 1 wherein the substituted urea is present in an amount from  $3 \times 10^{-3}$  to  $7.5 \times 10^{-2}$  grams per liter.

30

\* \* \* \* \*

35

40

45

50

55

60

65